

## UNITED STATES PATENT OFFICE

2,135,446

## PROCESS FOR TRANSFERRING MARKINGS

Herbert L. Wampner, Terre Haute, Ind., assignor  
to Commercial Solvents Corporation, Terre  
Haute, Ind., a corporation of Maryland

No Drawing. Application July 19, 1935,  
Serial No. 32,234

3 Claims. (Cl. 41—33)

My invention relates to the production of a coating material suitable for the reception of impressions by pressure transfer from pencilled markings and the like. More specifically, my invention relates to the production of a transfer lacquer for use in transferring pencil sketches and the like to the surfaces of blocks in the process of rubber block printing.

The process of rubber block printing involves the transfer of the original pen or pencil sketch to the surface of the rubber block, cutting the block to correspond to the transferred sketch and subsequently printing from the cut block. In the case of color printing, a separate block must be cut for each color, which means that the original sketch must be transferred successively to each block in order to secure perfect register. The problem of transferring a sketch to a series of blocks has not been successfully solved in the past. Various coating materials, such as lithograph varnishes, have been applied to rubber blocks for receiving impressions by pressure transfer, but these materials have been unsatisfactory, particularly from the standpoint of the critical time limit within which the transfer must be made. The standard practice in the art has, therefore, avoided the use of any such coating. Rubber blocks having a pronounced gray sulfur bloom are utilized for the purpose, and the pencil sketch is transferred directly to the gray surface by rubbing the back of the pencil lines with a hard rounded instrument. Such a procedure is fairly satisfactory for transfer to a single block. Even in this case, however, the procedure is disadvantageous from the standpoint that errors cannot be corrected, since the removal of the sulfur bloom from the surface of the block makes the block useless for further transfers. This procedure is also quite unsatisfactory for color printing, in which case numerous transfers must be made from a single sketch. A single transfer directly to the rubber block requires excessively hard rubbing and tends to stretch the paper on which the original sketch is made. Thus, after a series of transfers the original sketch is distorted and perfect register of the colored prints is unobtainable.

I have now discovered an improved coating material which may be applied to the surface of rubber blocks and the like for receiving impressions by pressure transfer, and which avoids all of these prior difficulties. This material comprises essentially a cellulose ester lacquer containing an unusually high percentage of plasticizer. The amount of plasticizer to be employed should be sufficient to maintain a dry film of the lacquer (i. e., a film free from volatile sol-

vents) in a pressure-imprintable state but insufficient to maintain such a film in a tacky state. For this purpose I have found that an amount of raw castor oil equal to about three times the weight of the cellulose ester imparts satisfactory properties to a nitrocellulose lacquer. Equivalent amounts of other plasticizers may be used, and in general it may be said that from 150 to 450% of a non-solvent plasticizer such as raw castor oil, or from 75 to 125% of a solvent plasticizer such as dibutyl phthalate, dibutyl tartrate, tricresyl phosphate, and the like, based on the weight of the cellulose ester, may be satisfactorily employed.

I have found that in the case of transfer lacquers for application to rubber blocks a solvent mixture should be employed which is free from hydrocarbons in order to prevent undue softening or swelling of the rubber. Transfer lacquers for this purpose should, therefore, be formulated with a solvent mixture of esters, ketones, alcohols, and the like which are chemically inactive to rubber. The usual solvent mixtures for the cellulose ester employed may be used, merely omitting the common hydrocarbon diluents.

My invention may perhaps best be illustrated by the following specific examples:

## Example I

| Solids                           | Grams per 100 ml.<br>of solvents | 30 |
|----------------------------------|----------------------------------|----|
| Nitrocellulose (film scrap)..... | 5                                |    |
| TiO <sub>2</sub> .....           | 10                               |    |
| Raw castor oil.....              | 15                               | 35 |

| Volatiles          | Percent by volume | 40 |
|--------------------|-------------------|----|
| Ethyl acetate..... | 20                |    |
| Ethyl alcohol..... | 65                |    |
| Butyl acetate..... | 15                |    |

## Example II

| Solids                           | Grams per 100 ml.<br>of solvents | 45 |
|----------------------------------|----------------------------------|----|
| Nitrocellulose (3/4 second)..... | 16                               |    |
| TiO <sub>2</sub> .....           | 20                               |    |
| Dibutyl phthalate.....           | 20                               | 50 |

| Volatiles          | Percent by volume | 50 |
|--------------------|-------------------|----|
| Ethyl acetate..... | 20                |    |
| Ethyl alcohol..... | 65                |    |
| Butyl acetate..... | 15                |    |

## Example III

|    | Solids                                     | Grams per 100 ml.<br>of solvents |
|----|--------------------------------------------|----------------------------------|
| 5  | Cellulose acetate (safety film scrap)..... | 5                                |
|    | TiO <sub>2</sub> .....                     | 10                               |
|    | Diethyl tartrate.....                      | 6                                |
| 10 | Volatiles                                  | Percent by volume                |
|    | Acetone.....                               | 80                               |
|    | Ethyl alcohol.....                         | 20                               |

- 15 The above lacquers may be thinned, prior to application, to the desired consistency for brushing or spraying. In general, a dilution of about 1:1 with a thinner of the same composition as the volatiles of the lacquer will be found to be satisfactory. After application and drying in the usual manner, the resulting films will be found to be highly satisfactory for the reception of impressions by pressure transfer from pencil or ink markings. The solvent free films (i. e., air dry films free from volatile solvents) will be found to be non-tacky but permanently receptive to pressure imprint. The term non-tacky in this connection has the usual meaning signifying the state in which a finger may be drawn lightly over the surface without feeling sticky. This state is often referred to also as "dust free" (Gardner, "Physical and Chemical Examination of Paints, Varnishes, Lacquers and Colors", Washington, D. C., 1930, page 296). The term pressure-imprintable as used herein also has the common meaning signifying the state in which full pressure of a finger leaves a permanent mark upon the film.
- 20 It will be seen that blocks coated with a material of these characteristics will have many advantages over materials previously available. The coatings are sufficiently resistant so that the blocks may be handled with reasonable care and stored in the usual manner without adversely affecting the treated surfaces. Also the coatings retain their pressure-imprintable character for a sufficient length of time for ordinary commercial usage including ordinary storage periods. This characteristic may, in fact, be termed practically permanent.
- 25 The coatings, which may be pigmented in a contrasting color from that of the sketch to be transferred yield sharp impressions with sufficiently light pressure so as not to stretch the paper and distort subsequent impressions. Any of the common materials may be employed for making the original sketch or tracing, such as ordinary pencil, indelible pencil, transfer inks, and the like. An ordinary soft lead pencil will produce satisfactorily as many as six or eight transfers. An indelible pencil will give twelve or more sharp impressions. It is, therefore, seen that a coating material of this type is highly satisfactory for use in preparing a series of blocks

for color printing. A further advantage lies in the fact that errors can readily be corrected by removing the lacquer with solvents and applying a new coating to the block. Other advantages of materials of this type will be evident from the preceding description.

It will be understood, of course, that my invention is not to be limited to the particular examples disclosed above. Various equivalent materials may be employed, and the nature of the lacquer may be modified by the addition of resins or other common ingredients of cellulose ester lacquers. A clear lacquer may be employed if the color of the base to which it is applied is satisfactory, or various pigments or dyes may be incorporated according to the nature of the transfer that is to be made. It will be evident that while my coating materials are especially adapted for application to rubber blocks, they may be satisfactorily employed for coating other objects for transfer use. Uses in wood block printing, linoleum printing, and the like, will readily suggest themselves to those skilled in the art. In such uses hydrocarbons could be included in the solvent mixture, and in any case a solvent mixture may easily be formulated to have minimum attack on the particular base employed. In general, it may be said that any modifications or equivalents which would naturally occur to one skilled in the art may be employed without departing from the scope of my invention.

My invention now having been described what I claim is:

1. A process for transferring markings from a sheet of paper, or similar thin material, to a solid surface which comprises applying to said solid surface a coating of a cellulose ester lacquer containing sufficient plasticizer to maintain a solvent free film of said lacquer in a pressure imprintable state, but insufficient to maintain such a film in a tacky state, drying said coating to a solvent free condition and transferring the markings from the said thin material to the resulting lacquer film solely by pressure transfer.

2. A process for transferring markings from a sheet of paper, or similar thin material, to a solid surface which comprises applying to said solid surface a coating of a cellulose ester lacquer containing from 150 to 450% of a non-solvent plasticizer based on the weight of the cellulose ester, drying said coating to a solvent free condition and transferring the markings from the said thin material to the resulting lacquer film solely by pressure transfer.

3. A process for transferring markings from a sheet of paper, or similar thin material, to a solid surface which comprises applying to said solid surface a coating of a cellulose ester lacquer containing from 75 to 125% of a solvent plasticizer based on the weight of the cellulose ester, drying said coating to a solvent free condition and transferring the markings from the said thin material to the resulting lacquer film solely by pressure transfer.

HERBERT L. WAMPNER. 65